

Jan. 10, 1928.

1,655,484

W. H. WHEELER

METHOD OF MANUFACTURING AUTOMOBILE IDENTIFICATION DEVICES

Filed Nov. 26, 1923

*Fig. 1.*



*Fig. 2.*



*Fig. 3.*



INVENTOR  
*William H. Wheeler*  
BY  
*Amelia Bond*  
ATTORNEY

Patented Jan. 10, 1928.

1,655,484

# UNITED STATES PATENT OFFICE.

WILLIAM H. WHEELER, OF GLEN RIDGE, NEW JERSEY, ASSIGNOR, BY MESNE ASSIGNMENTS, TO FEDCO NUMBER PLATE CORPORATION, OF NEW YORK, N. Y., A CORPORATION OF DELAWARE.

## METHOD OF MANUFACTURING AUTOMOBILE IDENTIFICATION DEVICES.

Application filed November 26, 1923. Serial No. 677,018.

This invention relates to an improved method of manufacturing automobile identification devices of the general character disclosed in my co-pending applications, 5 Serial Nos. 662,230 and 662,231, dated September 12, 1923.

In the foregoing applications, different methods have been described of producing vari-colored effects on the surface of an identification plate.

One of the above noted applications, namely, Serial No. 662,230, shows a plate embodying different colored effects, which have been produced by building up a composite plate of a number of sheets of different colored metals, and then subjecting said plate to a process whereby the various metals are caused to appear in different areas in the surface of the plate.

20 A somewhat different method of obtaining the desired colors has been shown in my application, Serial No. 677,017, dated November 26, 1923. In this instance, the color effects have been made to appear by first 25 heat-treating the plate at a temperature known to produce a certain colored oxide, and then after grinding off certain portions of such oxidized surface, again heat-treating the plate at a different temperature so as to 30 produce an oxide of a different color on the ground off surfaces without affecting the color of the first oxide.

The aim of the present invention is to 35 produce an identification plate having a multi-colored surface without resorting to the above noted methods of producing the same and to simplify the process of manufacture.

Another object of this invention is to 40 produce the plates in such a manner that they may be quickly and cheaply manufactured on a large scale and at the same time be very difficult to reproduce on a small scale by an unauthorized person without involving great 45 labor and the use of expensive apparatus.

It is a further object of the invention to 50 provide an identification device for use principally with automobiles and which will prevent in large measure the undetected theft thereof.

One practical embodiment of my invention is illustrated in the drawings forming a part of this application and in which:

Fig. 1 is a perspective view showing one of the stages in the formation of my identification plate, 55

Fig. 2 is a similar view showing another stage, and

Fig. 3 is a view of the finished plate.

Referring to the drawing by numerals, 60 10 indicates a plate of suitable proportions which is adapted to be secured to the frame or engine block of an automobile, the surface of the plate having been oxidized to produce a color thereon, indicated by 11. 65 Embossed numerals 12 are formed on the plate prior to the color treatment and in the next operation (Fig. 2) have their surfaces ground off so as to allow the original color of the plate metal to appear through the 70 background as at 13.

I have found that by subjecting the oxidized surface of a plate to pressure it is possible to change the color of said surface to a degree depending upon the amount of 75 pressure brought to bear thereon. I am unable to explain with any degree of certainty why said change of color takes place. However, I am inclined to believe that the color is altered by a physical or a structural 80 change. Since such portions of the plate as are under a greater pressure in the embossing operation, are rendered thinner than other portions, the thickness of the oxide is also rendered thinner. In other words, 85 there is an outward flow of metal from under the embossing die, which serves to spread the oxidized surface in such a way as to produce a change in its light reflecting surface, whereas the parts which are not subjected to so high a pressure are compacted 90 rather than spread out, so that the original color of the oxide is preserved and, if anything, intensified. I have found, for instance, that a nickel surface oxidized to give 95 a blue color, will, when subjected to pressure in the embossing die, change its color from blue to a brownish tone in the background portions of the embossed design, i. e., in those portions which are subjected to a 100 higher pressure. Utilizing this principle and by subjecting certain portions of the surface area of a plate to the pressure of an embossing tool, I have produced a raised design of the original color on the portions 105 15, not under pressure, and a contrasting

background of a different shade on the sunken portions 16 which have been under pressure.

Thus, it will be seen that an embossing operation and color changing process are performed at the same time, doing away with steps heretofore found necessary in producing a plate of this character.

The cost of manufacture has been consequently reduced and the production problem very much simplified.

The finished product disclosed in Fig. 3 embodies a two color effect comprising dark

embossed areas 15 and the lighter background 16. The numerals 12 which are of 15 the natural color of the plate metal contrast sharply in color with both against the background and the embossed design.

I claim:

A process of producing a vari-colored 20 embossed plate which consists in oxidizing a plate, and subjecting the plate to an embossing operation under a pressure sufficient to change the color of the more deeply impressed parts of the plate surface.

WILLIAM H. WHEELER.